

Sept. 7, 1948.

A. H. DAVIS

2,448,782

COMPOSITE STRAND AND FABRIC

Filed May 14, 1945

Fig. 1.



Fig. 2.



Fig. 3.



Fig. 4.



Fig. 5.



Fig. 6.



Fig. 7.



Fig. 8.



Inventor:

Archibald H. Davis

234

Pierce + Scheffler

Attorneys.

## UNITED STATES PATENT OFFICE

2,448,782

## COMPOSITE STRAND AND FABRIC

Archibald H. Davis, Washington, D. C.

Application May 14, 1945, Serial No. 593,693

4 Claims. (Cl. 57—140)

1

This invention relates to novel composite textile strands and to textile fabrics made therefrom including woven, knitted, plied and laminated sheets, webbing, belts, tapes, cordage and the like.

A general object of the invention is the provision of composite textile strands and fabrics including fibers of high tensile strength, high resistance to atmospheric influence and to biological attack, and high heat stability and having likewise a high degree of adhesiveness to coating and laminating compositions.

While materials such as siliceous, nylon and fine metallic fibers possess in high degree the strength, resistance and stability desired in many cases, particularly in industrial applications, these fibers are all characterized by relatively smooth non-adhesive surfaces which entail serious disadvantages in the use of fibers of this type.

I have found that by suitably combining high strength fibers of low surface adhesion with organic plastic fibers, it is possible to provide composite strands and fabrics in which the adhesion of the components is greatly increased without any sacrifice of the strength and resistance properties of the high strength fibers.

In general, the invention includes composite textile strands comprising an organic plastic fiber and at least one high strength fiber of low surface adhesion, such as glass, nylon, or metal, disposed about the organic plastic fiber in contact with a portion only of the surface of the organic plastic fiber, whereby the adhesive properties of the strand is greatly increased not only by the adhesiveness of the organic plastic fiber but by the effective mechanical interlocking provided by the channels and projections embodied in the strand and fabric construction. The invention also includes textile fabrics broadly, woven, knitted, plied and laminated from the strands of the invention into sheets, webbing, belts, tapes, cordage and the like which may be coated, laminated or otherwise treated to produce articles of improved utility or appearance.

Typical of the high strength fibers of low surface adhesion useful in the invention are glass fibers produced in the known way of any desired dimensions, composition and color. Other high strength fibers suitable for use in the invention are asbestos fibers, mineral wool fibers, nylon fibers, and metallic fibers or wires.

The organic plastics useful in the invention may be selected from a wide variety of classes of organic resins and elastomers including cellulose esters and ethers; polymerization and copolymerization products of olefinic compounds,

2

such as vinyl compounds, styrene, acrylic acid and its derivatives; synthetic or artificial rubber compositions, such as polymerized dienes and the various modifications thereof, rubber halides and hydrohalides, and chloroprene; urea-, thiourea-, and melamine-aldehyde resins; phenol-aldehyde resins; glycerol-polybasic acid resins; polycarboxylic amide condensation products; and mixtures of two or more resins or elastomers. The plastics may include suitable plasticizers, pigments, fillers and other modifying agents well known in the plastic art.

The composite strands of the invention may be made in a wide variety of ways, such as by plying or twisting together one or more threads or fibers of high strength material of relatively low surface adhesion.

The strands may be so formed that either the high strength fibers or the organic plastic fibers project in the strand beyond the effective diameter of the other fibers in the strand in accordance with the use to which the strands are to be put.

In forming the strands by twisting, the relative tensions on the high strength fibers and on the plastic fibers may be adjusted with respect to the relative diameters of the fibers to cause either of the fibers to overlie the other in the strands as may be desired. The amount of projection of the organic plastic fiber in the strand section may be increased after formation of the strand by a suitable treatment such as by heating or by treating with a suitable swelling agent. The fibers may be twisted or plied in a multiple of directions in the strand. The strand and fabric construction of the invention is thus subject to a wide variation without departing from the characteristic principle of the invention that the composite strands and fabrics of the invention present interspersed and interlocking surfaces of both the high strength fiber and the organic plastic fiber.

The invention will be more particularly described with reference to the accompanying drawing showing illustrative embodiments of the principles of the invention.

Fig. 1 is an enlarged diagrammatic representation of a composite strand embodying the principles of the invention;

In the drawing:

Figs. 2, 3, 4, 5 and 7 are enlarged diagrammatic representations of further embodiments of the invention;

Fig. 6 is an enlarged diagrammatic section of a coated fabric embodying the composite strand of Fig. 5, and

Fig. 8 is an enlarged diagrammatic section of

a coated fabric embodying the composite strand of Fig. 7.

In the strand shown in Fig. 1, the high strength fiber 10 and the organic plastic fiber 11 are of substantially the same diameter. As shown in the fiber, the high strength fiber 10, of glass, for example, is caused to project to a greater diameter in the strand by giving it a greater degree of twist, for example, by subjecting the plastic fiber to greater tension than the high strength fiber while twisting the two fibers into the strand.

In the strand of Fig. 2, the high strength fiber 10 has a greater fiber diameter than the organic plastic fiber 11 so that when twisted into a strand at substantially the same tension the high strength fiber projects to a greater distance in the strand than the plastic fiber.

In the strands of both Figs. 1 and 2, the relative positions of the fibers in the strand may be reversed. In the forms shown, the mechanical interlocking effect in fabric structures and in coated constructions is more predominant than when the organic plastic fiber is outermost in the strand.

In the strands of Figs. 3 and 4, high strength fibers or wire 10 are plied or twisted about substantially straight organic plastic fibers 11. A plurality of high strength fibers 10 of different directions of twist may be utilized as in Fig. 4.

Fig. 5 shows a strand having six high strength fibers 10 plied about a relatively straight organic plastic fiber 11 of substantially greater fiber diameter.

Fig. 6 shows diagrammatically the combined adhesive and mechanical interlocking effect of the strands of Fig. 5 when combined into a fabric and coated with a coating composition 12.

Fig. 7 shows a strand having three high strength fibers 10 plied about an organic plastic fiber 11 of substantially smaller fiber diameter.

Fig. 8 shows the strands of Fig. 7 composed into a coated fabric construction combining high strength and a high degree of cohesion of the fabric elements the coating composition being indicated at 12.

The strands of the invention in their various forms adapt themselves to plying, knitting, weaving and the like into fabric structures of a wide variety of patterns. For example, by weaving the strands into a ribbed fabric structure both the structure of the strands and the fabric structure itself cooperate to increase adhesion and mechanical interlocking in coated and laminated structures.

It will be clear from the foregoing construction and examples that the construction and arrangement of the strands and fabrics may be widely varied without departing from the prin-

ciples of the invention as defined in the following claims.

I claim:

1. A composite textile strand comprising an organic plastic fiber and at least one glass fiber intertwisted therewith in contact with a portion only of the surface of the organic plastic fiber, the relative twist of the glass fiber being greater than that of the organic plastic fiber by an amount sufficient to project the glass fiber to the periphery of the strand.

2. A composite textile strand comprising an organic plastic fiber and at least one glass fiber of lesser fiber diameter than the organic plastic fiber intertwisted therewith in contact with a portion only of the surface of the organic plastic fiber, the relative twist of the glass fiber being greater than that of the organic plastic fiber by an amount sufficient to project the glass fiber to the periphery of the strand.

3. A textile fabric comprising a plurality of strands including an organic plastic fiber and at least one glass fiber intertwisted therewith in contact with a portion only of the surface of the organic plastic fiber, the relative twist of the glass fiber being greater than that of the organic plastic fiber by an amount sufficient to project the glass fiber to the periphery of the strand, and a coating composition bonded to the glass fibers of the fabric by contact with the organic plastic fibers.

4. A textile fabric comprising a plurality of strands including an organic plastic fiber and at least one glass fiber of lesser fiber diameter than the organic plastic fiber intertwisted therewith in contact with a portion only of the surface of the organic plastic fiber, the relative twist of the glass fiber being greater than that of the organic plastic fiber by an amount sufficient to project the glass fiber to the periphery of the strand, and a coating composition bonded to the glass fibers of the fabric by contact with the organic plastic fibers.

ARCHIBALD H. DAVIS.

#### REFERENCES CITED

The following references are of record in the file of this patent:

#### UNITED STATES PATENTS

| Number       | Name     | Date          |
|--------------|----------|---------------|
| 2,110,979    | Rider    | Mar. 15, 1938 |
| 2,217,826    | Van Laer | Oct. 15, 1940 |
| 2,252,999    | Wallach  | Aug. 19, 1941 |
| 55 2,306,781 | Francis  | Dec. 29, 1942 |
| 2,313,058    | Francis  | Mar. 9, 1943  |
| 2,313,104    | Wallach  | Mar. 9, 1943  |
| 2,335,644    | Camp     | Nov. 30, 1943 |